

## UNITED STATES PATENT OFFICE

2,013,841

## MANUFACTURE OF FIBER ARTICLES

George A. Richter, Berlin, N. H., assignor to  
 Brown Company, Berlin, N. H., a corporation of  
 Maine

No Drawing. Application December 10, 1932,  
 Serial No. 646,741

5 Claims. (Cl. 92—20)

This invention relates to the manufacture of fiber articles whereinto cellulose pulp enters as raw material. While not restricted thereto, it relates more particularly to the manufacture of so-called water-laid felts designed for impregnation purposes and formed on machinery of the paper-making type.

In the manufacture of fiber articles, such as water-laid felts, intended for impregnation purposes, it is frequently desirable that the pulp used as raw material be in a substantially unhydrated or "free" condition. Otherwise, the hydrated or gelatinized cellulose tends to bind together the pulp fibers of the article into which the pulp is formed and, although enhancing the strength, tear resistance and other physical qualities of the article, detracts from its absorptive capacity, i. e., from the amount of impregnant which the article takes up and from the speed and uniformity with which the impregnant diffuses into and throughout the article. Moreover, despite the fact that a fiber article may be possessed of good strength, tear resistance and other physical qualities by virtue of the fact that its pulp component has been hydrated or gelatinized, nevertheless, it has been established that it is those articles whose pulp component has been kept in a substantially unhydrated or free condition that acquire the best physical qualities after they have undergone impregnation with a given impregnant. For instance, water-laid felts made from cellulose pulp which has been preserved in as free a condition as possible, may be quite tender and lacking in tensile strength, tear resistance, and other qualities to begin with, but when they are impregnated with various binders such as asphalt, rubber and the like, they acquire remarkable toughness, body, strength, tear resistance, and other valuable physical properties. Again, they can imbibe quickly and uniformly a high percentage of impregnant.

There are various cellulosic stocks which may serve as the starting material for the production of pulps or halfstuffs adapted for conversion into waterlaid felts or other fiber articles. Some of these raw materials, notably rags, rope stock or the like, have to be reduced or disintegrated in water in a so-called hollander or beater engine before the long fibers, yarns, or cloth constituting such materials have been resolved into fiber units which can form or interfelt uniformly and otherwise satisfactorily on machinery of the paper-making type, e. g., a felt-forming machine. In other words, the cellulosic stock must undergo mechanical fiber-liberating or pulping action in

the presence of water before it can be satisfactorily formed into such articles as water-laid felts. The subjection of rags, rope stock or similar cellulosic material to beater action, however, is inevitably accompanied by the hydration or gelatinization of the pulp thereby prepared, wherefore, the conditioned pulp or halfstuff rather than being a free one, possesses a comparatively high "slowness" and accordingly leads to felts of a relatively dense and "boardy" character.

In accordance with the present invention, a cellulose pulp or halfstuff which has been hydrated or gelatinized by virtue of beater action upon rags, rope stock or similar cellulosic material, is transformed into a free pulp or halfstuff by treatment with suitable chemicals which dissolve or otherwise destroy the hydrated or gelatinized cellulose or other components imparting slowness to the pulp or half-stuff. While various chemicals might be used for the purpose of destroying the hydrated or gelatinized cellulose present in the pulp, I prefer to use alkaline reagents of such a type and under such conditions as will ensure the destruction of the hydrated or gelatinized cellulose without sensibly damaging the pulp fibers. Indeed, by the selection of the appropriate alkaline compound and treating conditions, it is possible to destroy the undesirable hydrated or gelatinized cellulose while at the same time improving the pulp fibers for formation into water-laid felts or other fiber articles designed to undergo an impregnating treatment. Thus, the hydrated or gelatinized cellulose may be destroyed while enhancing the absorbency and purity of the pulp fibers so that water-laid felts made from the pulp lend themselves better to impregnation not only because they are essentially free from undesirable cellulosic binding or cementing ingredients, but because the pulp fibers themselves are soft and absorbent and so contribute such qualities to the felts in which they exist.

There are various ways in which the principles of the present invention may be availed of and there are various kinds of cellulosic materials to which these principles may be applied to greater or less advantage. Inasmuch as rag stock constitutes a form of cellulose in connection with which the present invention may, so far as I am now aware, be practiced to greatest advantage, I shall describe specifically the conditioning of rag stock in accordance with my invention for the preparation of water-laid felts. Thus a rag stock such as is commonly used as raw material in the manufacture of roofing or floor-covering

felts, may constitute my starting material. If desired, the rags may be cut or shredded while substantially dry into the smallest pieces or cloth fragments economically producible in this way, 5 thereby minimizing the work that need be done by the beater engine and hence minimizing the generation of hydrated or gelatinized cellulose during the beating operation. The rags in a normal or reduced condition may then be delivered 10 into a hollander or beater engine together with sufficient water to ensure circulation and the beater roll may be run in the usual cutting relationship with the bed-plate until the rags have been reduced to a pulp or halfstuff which 15 can be formed into a felt which is satisfactory from the standpoint of uniformity of texture and smoothness of surface. Inasmuch as the resulting pulp or halfstuff will normally be a dilute aqueous pulp suspension, that is, have a fiber content of about 5% or less, as does the usual beaten stock, it may be desirable to thicken or partially 20 dewater the beaten pulp before it undergoes the action of a chemical which destroys in large measure or practically entirely its hydrated or gelatinized cellulose constituent. To this end, the beaten pulp may be delivered to thickeners or other dewatering instrumentalities which raise its fiber content to, say, about 10% or greater. The pulp thus thickened may then be treated 25 with an alkali under suitable conditions of alkalinity and temperature to effect the desired change in the properties of the pulp.

According to one procedure, the thickened pulp is boiled in dilute caustic soda solution, say 30 one of about 1% to 3% strength under atmospheric or superatmospheric pressure for about one to three hours, whereupon the pulp is washed free of alkaline liquor. The washed pulp is characterized by its high freeness and softness. According 35 to a second procedure, the pulp may be treated at or below room temperature conditions with a caustic soda solution of greater strength, say, one of about 5% to 8% soda concentration, for about 30 minutes to 2 hours, and then washed. In such case too, the hydrated cellulose is dissolved or destroyed and the pulp fibers transformed into a soft, absorbent condition. According 40 to a third procedure, the pulp may be subjected to the action of a caustic soda solution of mercerizing activity at or below room temperature conditions. At about room temperature, 20° C., a solution of about 18% or greater strength has full mercerizing activity, but inasmuch as such activity exists to some extent in solutions of 45 as low as about 10% strength at room temperature, such latter solutions may also be considered for the purposes of my invention as having mercerizing activity. At lower than room temperature, say at 5° C., or at 0° C., solutions of lower 50 causticity than 10% caustic soda strength are characterized by their ability to mercerize cellulose fiber and to destroy hydrated cellulose associated therewith. It is thus possible to employ various conditions of causticity and temperature 55 in the caustic soda solution to which the pulp is exposed in order to realize the transformation of the pulp to the condition desired in accordance with my invention. When strong caustic soda solutions are employed for the treatment of the 60 pulp, as hereinbefore described, the liquor may be separated from the pulp as in a counter-current washer designed to effect washing of the pulp with minimum dilution of the liquor so that the separated liquor may be re-used in the treatment 65 of other pulp. If desired, rather than

washing the stock free from the liquor, the excess liquor may be separated without dilution as in a centrifuge, thickener, or other separating apparatus. A portion of the liquor may thus be recovered in an undiluted condition and be reused with little, if any, fortification in the treatment of other pulp. The centrifuged or thickened pulp may then be washed free of the residual liquor, as hereinbefore described. When the pulp is treated with a refrigerated caustic soda solution, for instance, one at 0° to 5° C., mercerization 70 may be effected with a caustic soda solution containing as little as 5% caustic soda. It is in fact possible to operate at temperatures below the freezing point, in which case mercerization may be effected with even more dilute caustic soda solution as in such case ice or water crystals separate out from the solution, in consequence of which the unfrozen or liquid portion of the solution becomes more concentrated in caustic soda 75 and functions more effectively as a mercerizing agent. In the event that the treatment of the pulp is performed with a refrigerated or partially frozen mercerizing liquor, it is of decided advantage to separate out the excess refrigerated liquor from the pulp so as to conserve it in a refrigerated as well as undiluted condition for the treatment of other pulp. Should a portion of the mercerizing liquor be frozen, it may be thawed out to permit a separation of as much liquor as possible 80 from the pulp before the pulp is washed.

The alkaline liquor used for the purpose of the present invention may have its alkalinity furnished in whole or in part by alkalies other than caustic soda. For instance, when the treatment 85 of the pulp is performed more particularly at elevated temperature, the liquor may have its alkalinity furnished by sodium sulphide, sodium carbonate, lime, sodium borate, sodium phosphate, sodium sulphite, or like salts, which undergo 90 hydrolysis in water to yield an alkaline aqueous medium. Some of these salts, like the borates, phosphates, and sulphites, may require the use of higher treating temperatures to give the same effect as that attainable through the use of caustic soda, sodium sulphide and sodium carbonate at lower temperatures. It is of course possible to use various combinations of alkalies or salts 95 which give an alkaline aqueous medium. For instance, the so-called white liquor of a kraft pulp mill, which as is well known, contains sodium sulphide as well as caustic soda, may in some instances be advantageously employed, either under mercerizing or under non-mercerizing conditions. The alkaline liquor may, if desired, contain suitable 100 oxidants such as hypochlorite bleach, sodium peroxide, hydrogen peroxide, permanganate, or the like, particularly when it is strongly alkaline or is used under mercerizing conditions. An oxidant should not, however, be used in an alkaline liquor when a reducing agent like sodium sulphide is present therein. An alkaline liquor containing an oxidant is of value more particularly in connection with a colored pulp, as it makes possible partial or complete decolorization 105 of the pulp. The fact is that in some cases it may be advantageous to treat the rags or other starting material before they undergo beater action or while they are undergoing beater action with oxidants such as chlorine, hypochlorite 110 bleach, permanganate or the like, and then to wash the pulp before it is treated with an alkaline liquor containing, if desired, additional oxidant.

In some instances, the rags may be cooked in an 115

alkaline liquor and/or chlorinated or bleached prior to beating. In other instances, the beaten stock may be chlorinated or bleached and then treated with alkaline liquor, as hereinbefore described, to destroy hydrated cellulose present therein; or the beaten stock may be treated with alkaline liquor, as hereinbefore described, to destroy hydrated cellulose present therein and then bleached. The stock is preferably washed between the bleaching and alkaline treatments. It is of course possible to apply the foregoing chemical treatments in other combinations or sequences, but in each case, the principle of destroying hydrated cellulose generated during the beating operation is utilized, thereby increasing the freedom of the pulp or halfstuff after the beating operation. I may, however, state that it is preferable to carry out such alkali treatment as is desired or necessary only after the beating operation so as to refine or purify the pulp at the same time as its hydrated cellulose constituent is being destroyed. The chlorinating or bleaching treatment may, however, advantageously be performed on the raw rags, as such treatment tends to promote subsequent disintegration in the beater engine, whereas an alkali treatment of refinement of the rags, as by cooking in alkaline liquors, works the other way, that is, tends to diminish ease of disintegration in the beater engine. If desired, however, the chlorinating or bleaching treatment may be performed partly before beating and partly after beating; or it may be performed in entirety after the beating operation, whereupon the rag pulp may then have its hydrated cellulose ingredient destroyed by the action of an alkaline liquor which may simultaneously serve to remove oxy cellulose or other undesirable products formed during bleaching and otherwise to refine or purify the pulp. As already indicated, the rags may be preliminarily cut or shredded in a dry way to facilitate subsequent chemical treatment as well as beating.

When pulp or halfstuff containing hydrated or gelatinized cellulose is processed in accordance with any one of the foregoing procedures of my invention, it is rendered so free that when made into felts on the usual felt-making machines, the felts are comparatively tender or lacking in tensile strength and tear resistance and are highly porous, bibulous, soft and flexible. Notwithstanding the fact that such felts are thus poor in their physical qualities as unimpregnated felts, they can be impregnated quickly and uniformly with various binders such as latex, natural and synthetic resins, cellulose ester solutions, waxes, bitumen, or other binders of a thermoplastic, water-dispersed or dissolved variety, to form impregnated products of a high binder content and characterized by a highly desirable combination of characteristics. The felt may, for example, be bituminized to form a sheet which is highly pliant and practically proof against tear, especially the initiation of tear, and hence highly valuable in the roofing and felt base floor covering industries, for example. It becomes leatherlike in its properties when impregnated with rubber latex, rubber solutions or the like, and then dried. Apparently, the fact that the contiguous fibers in the felt are not bonded strongly by a hydrated or gelatinized cellulose is responsible for the high tear resistance in a bituminized sheet, for example, since it is quite likely that when a tearing stress is applied to the sheet, the stress rather than becoming localized and giving rise to rupture of the sheet, is not confined to any particular

locus, but it is distributed and/or dissipated over a large area on account of the freedom of the fibers to slip or move past one another.

In making the water-laid felts or foundations of the present invention, it may be of advantage to admix with the free pulp or halfstuff a suitable small proportion of pulp in a partially hydrated or well hydrated condition. The well hydrated pulp may be prepared by beating rag stock as hereinbefore described or by over-beating such stock or other suitable cellulose fiber in much the same way as is done in connection with the manufacture of glassine papers. The best kinds of hydrated or gelatinized cellulose for blending with the free pulp or halfstuff is that prepared in a so-called stone-rolled beater from kraft or other wood pulps refined by alkali to higher alpha cellulose content. In connection with pulps which have been rendered free by the use of caustic soda solutions of mercerizing activity, it is desirable to use a suitable proportion of unmercerized cellulose pulp which may be in a substantially unhydrated, partially hydrated or well hydrated condition. The use of some unmercerized pulp together with the mercerized pulp facilitates the production of uniformly textured felts, serving to offset the clumping or bunching tendencies in mercerized pulp. It is, however, possible to avoid clumpy or non-uniform felt formation even when the entire felt-making furnish is mercerized by delivering the furnish in an extremely dilute and well mixed condition to the felt-forming machine. The use of hot water as a suspending medium for the mercerized pulp also mitigates the clumping or bunching tendencies of the mercerized fibers.

It is to be observed that in accordance with my invention, the beating of rags, rope stock or other similar cellulosic materials, which shall be designated in the appended claims by the generic expression "rag stock" and which must be reduced to fibers of the appropriate size for uniform felting on machinery of the paper-making type, is practiced in water containing little, if any, alkali. While it may be possible to inhibit the generation of hydrated or gelatinized cellulose by using a large amount of alkali in the water in which beating is being effected, nevertheless, the presence of considerable alkali in the beater water would interfere seriously with the rate at which the rags or similar cellulosic material would undergo disintegration, cutting or reduction into the desired kind of pulp or halfstuff and would greatly increase the power consumption and time of beating. Apparently, the alkali greatly softens the fibrous material, makes it more resilient, and reduces the effectiveness of the cutting edges of the beater roll. Again, an alkali, such as caustic soda, evidently reduces the coefficient of friction between the cutting edges of the beater roll and the fibrous material. I have observed, for example, that it is much more difficult to reduce refined rag stock, for instance, rag stock which has been mercerized, than unrefined rag stock into a pulp or halfstuff even though substantially all of the alkali has been removed from the refined or mercerized rag stock before it is subjected to beater action. By adopting the practice of the present invention, it is possible to take advantage of the ease with which unrefined rag stock can be reduced to a pulp or halfstuff in the beater engine and then to destroy through the use of a suitable chemical reagent, preferably alkali, the undesirable constituents and more especially the hydrated or gelatinized cellulose present in the resulting pulp or halfstuff.

I claim:—

1. A process which comprises partially bleaching rag stock whose fibers must be reduced in size in order to be uniformly feltable, beating the partially bleached rag stock in the presence of water to form a hydrated uniformly feltable pulp or halfstuff, bleaching the beaten pulp, thereafter treating the bleached pulp with an alkaline liquor to destroy hydrated cellulose and thereby to increase its freeness without sensibly damaging the pulp fibers, washing the treated pulp, and, without substantial subsequent beating of the fibers forming the resultant pulp with its fibers at essentially the same length as after the beating operation, into a waterlaid felt.
2. A process which comprises bleaching rag stock whose fibers must be reduced in size in order to be uniformly feltable, beating the bleached rag stock in the presence of water to form a hydrated, uniformly feltable pulp or halfstuff, thereafter treating the beaten pulp with an alkaline liquor to destroy hydrated cellulose and thereby to increase its freeness without sensibly damaging the pulp fibers, washing the treated pulp, and, without substantial subsequent beating of the fibers, forming the resultant pulp with its fibers at substantially the same length as after the beating operation, into a waterlaid felt.
3. A process which comprises beating ray stock whose fibers must be reduced in size in order to be uniformly feltable, in the presence of water to form a hydrated, uniformly feltable pulp or halfstuff, bleaching the beaten pulp, thereafter treating the bleached pulp with an alkaline liquor to destroy the hydrated cellulose and thereby to increase its freeness without sensibly damaging the pulp fibers, washing the treated pulp, and, with-

out substantial subsequent beating of the fibers, forming the resultant pulp with its fibers at essentially the same length as after the beating operation, into a waterlaid felt.

4. A process of producing a waterlaid felt which comprises beating rag stock, whose fibers must be reduced in size in order to be uniformly feltable, in the presence of water to form a hydrated, substantially uniformly feltable pulp or halfstuff containing the fibers in substantially their final 10 felt-making size, thereafter treating the pulp with an alkaline liquor to destroy hydrated cellulose and thereby to increase the freeness of the pulp without sensibly damaging the pulp fibers, washing the treated pulp, and, without hydrating 15 of the pulp thereafter, forming the resultant freer pulp, with its fibers at essentially the same length as after the beating operation, into a waterlaid felt.

5. A process of producing a waterlaid felt 20 which comprises beating rag stock, whose fibers must be reduced in size in order to be uniformly feltable, in the presence of sufficient water to form a hydrated, substantially uniformly feltable pulp or halfstuff of a fiber content downwards of 25 about 5% and containing the fibers in substantially their final felt-making size, thickening the hydrated pulp to a fiber content of at least about 10%, thereafter treating the thickened pulp with an alkaline liquor to destroy hydrated cellulose 30 and thereby to increase the freeness of the pulp without sensibly damaging the pulp fibers, washing the treated pulp, and, without hydration of the pulp thereafter, forming the resultant freer pulp, with its fibers at essentially the same length 35 as after the beating operation, into a waterlaid felt.

GEORGE A. RICHTER.